

Jan. 17, 1928.

1,656,270

C. R. DOWNS ET AL

COAL CLEANING

Filed May 8, 1925



Charles R. Downs Inventor  
Charles H. Strange  
By their Attorneys  
Ward, Crosby & Smith

## UNITED STATES PATENT OFFICE.

CHARLES R. DOWNS, OF NEW HAVEN, CONNECTICUT, AND CHARLES H. STRANGE, OF POTTSVILLE, PENNSYLVANIA, ASSIGNEES TO HIRSCH-LEDERER SYNDICATE, INC., OF NEW YORK, N. Y., A CORPORATION OF DELAWARE.

## COAL CLEANING.

Application filed May 8, 1925. Serial No. 28,776.

Our invention relates to coal cleaning. In order to remove slate and other impurities from coal as it comes from the mine, it has been suggested to screen out the silt and then subject the mixture of coal, slate, etc., to a gravity separation. For this purpose a fluid mass having a specific gravity intermediate the specific gravity of the coal and the specific gravity of the impurities, is used and the mixture supplied thereto whereupon the coal rises and floats near the top of the fluid mass and the heavier impurities sink in the same. In order to provide such a fluid mass, a mixture of water and sand has been suggested, the proportions of water and sand being so adjusted as to bring the specific gravity of the fluid mass to a value between that of the specific gravity of the coal and that of the specific gravity of the slate or other impurities. The fluid mass is kept in agitation in order that the specific gravity of the same may remain substantially uniform throughout the entire mass. The use of a dissolved soluble material to produce a fluid of sufficiently high specific gravity to float the coal and allow impurities such as slate to sink has been suggested, but has not proved commercially successful, and a fluid mass comprising a mixture of sand in water has proved the more advantageous. In such method the coal is drawn off at the top of the fluid mass with more or less of the water and sand, while the slate is drawn out separately from the bottom of the fluid mass also with considerable water and sand. Therefore, fresh sand and water must be continuously supplied in order to keep the volume and specific gravity of the fluid mass up to the necessary amount. The slate or similar impurities which are drawn off from the body of the fluid mass with considerable sand and water are separated therefrom by washing screens and the sand returned to the cycle. Also the coal which is drawn off from the top of the fluid mass with more or less of the sand and water, is separated therefrom by washing screens and the sand returned to the cycle. In the coal to begin with, there is considerable finely divided coal or coal dust and also a certain amount of degradation of the coal takes place during the process which thus produces some finely divided coal, which is too fine to be sepa-

rated from the sand on the screens and passes through the screens with the sand. Therefore, this finely divided coal or coal dust is returned to the fluid mass along with the sand. As the proportion of fine coal or coal dust in the fluid mass thus increases, a condition is reached where the specific gravity of the fluid mass (due to the accumulation of fine coal therein of relatively low specific gravity) is reduced to a point so that the fluid mass no longer efficiently floats the coal in order to separate it from the slate and similar impurities. Therefore it has been the practice at short intervals and after the fluid mass has thus become degraded by the inclusion of fine coal, to allow the fluid mass containing sand and finely divided coal to run to waste and introduce fresh clean sand to form the fluid mass in order to maintain the proper specific gravity of the fluid mass.

The cost of such sand replacement is a very important matter especially with coal which tends to form an appreciable amount of dust and also the finely divided coal or coal dust is lost. A similar loss of value also takes place even if other materials or other liquids are used to produce the fluid mass.

The main object of our invention is to substantially avoid these losses and thus render the process less expensive and more efficient. And for this purpose the finely divided coal or the coal dust or a substantial amount thereof are separated from the sand or the like which flows out from the fluid mass and after such separation the purified sand is returned to the fluid mass while the separated coal dust is obtained as a valuable by-product.

Further and more specific objects, features and advantages will more clearly appear from the detail description given below taken in connection with the accompanying drawings which form a part of this specification. In the drawings, Fig. 1 is a diagram illustrating a system for carrying out our improvements in one form thereof and Fig. 2 is a diagrammatic detail illustrating a modification.

Referring to Fig. 1, the run of mine coal is run from chute 1 onto a screen 2 in order to separate the silt therefrom, the silt falling into a hopper 3 while the remaining coal

with such impurities as slate and the like is fed onto chute 4 and into the conical gravity separator 5. The separator 5 is provided with a stirrer shaft 6 having thereon stirrer 5 blades 7 in order to keep the fluid mass in the vessel 5 agitated. The mixture of sand and water in the separator 5 is of such specific gravity that the coal will float in or at the top thereof while the slate or other 10 heavy impurities sink to the bottom and the gate valve 8 being open, these impurities with considerable sand and water fall into the trap 9. The coal which floats in or at the top of the separator 5 flows off through 15 a trough 10 and on to separating screens 11, 12 and 13 which classify the coal according to size and from the screens 11, 12 and 13, the classified coal is removed by chutes 14, 15 and 16 respectively. The sand and 20 water and also the fine coal dust or finely divided coal which is too small to be retained by the screens, passes therethrough into the hopper 17.

Periodically the gate valve 8 is closed and 25 the gate valve 18 at the bottom of the trap 9 is opened permitting the charge of slate, etc., sand and water in the trap 9 to be deposited on a separating screen 19 which permits the sand and water to pass therethrough into hopper 30 per 20 while the slate and similar impurities are removed on chute 21. The sand and water so separated is deposited in the settling tank 22 in which the sand settles to the bottom and the excess water flows off through 35 overflow 23. This sand which now contains very little impurities is pumped back by centrifugal pump 24 through pipe 25 and returned to the fluid mass in the separator 5 and also fresh water is introduced into the 40 fluid mass in separator 5 through pipe 26 in order that the volume of the fluid mass in the separator 5 may be kept at the desired height so that the coal will run off through the trough 10. The amount of water introduced 45 through pipe 26 and the amount of sand introduced through pipe 25 is so regulated as to keep the gravity of the fluid mass at the desired value.

The sand and water containing more or 50 less finely divided coal, from the screens 11, 12, 13 is led from the hopper 17 through pipe 27 to the bottom of a flotation separating apparatus 28. This apparatus 28 may be of any suitable or well known kind, operating in any suitable or well known manner to separate the finely divided coal from the sand which is preferably effected with the aid of a froth flotation agent, i. e. by the use of a relatively small quantity of oil or 55 frothing agent as distinguished from the use of a relatively large quantity of oil, which latter method is commonly known in the art as "bulk" oil flotation, while the former method using a relatively small quantity of 60 oil or other flotation agent is commonly

known as froth flotation. However the bulk oil flotation may be found advantageous in certain cases. The frothing agent may be introduced at the bottom of the apparatus 28 and also air under pressure may be introduced at the bottom of the apparatus in order to aid in the separation. Likewise other chemicals may be introduced to aid in the separation. In Fig. 1 the apparatus is shown with an agitator 31 in the lower part thereof whereby the mass is agitated in the bottom part of the cell, but suitable baffle plates as at 29 and 30 are provided whereby the mass in the upper part of the cell remains relatively quiescent. The 75 finely divided coal rises to the top of the apparatus 28 and flows out at the top thereof and may be removed through trough 32. The purified sand with water is removed from the bottom of the apparatus in any 80 suitable or well known manner and delivered to the settling tank 22 by pipe 33. From the above it will be seen that not only is the sand which is drawn off with the slate etc., saved and returned to the process, but 85 also the sand which is drawn off with the coal is saved and purified before it is returned to the fluid mass in the separator 5 whereby the fluid mass in the separator 5 is kept sufficiently free from finely divided coal 90 so that its specific gravity is kept up to the necessary point, all of which not only results in a substantial saving of sand, but also in a saving of substantial quantities of fuel values in respect of the finely divided coal which 95 is obtained from the froth flotation apparatus 28.

With regard to the sand and water which falls through the screens 11, 12 and 13, we believe that most of the finely divided coal 100 is found at the right hand end of the hopper 17, as viewed in Fig. 1 while the sand and water which come through the screen 13 at the opposite or left hand end thereof is relatively free from finely divided coal or 105 coal dust. Therefore this latter portion may need no further purification. And in order to avoid the waste of energy etc. in purifying such sand, the arrangement shown in Fig. 2 110 may be used wherein the hopper 17 only extends under the right-hand end of the screen 13 where it collects substantially all of the sand and water which is polluted with coal dust and delivers same to the froth flotation apparatus 28 by pipe 27. A separate hopper 115 35 is provided to receive the relatively pure sand and water from the opposite end of the screen 13 and this may be delivered directly to the settling tank 22 by means of pipe 36.

In order that the invention may be more 120 clear to those skilled in the art, we will give a specific example of the method as actually carried out. Run of mine of anthracite coal was passed over wet screens and then passed 125 into the separator containing the fluid mass 130

of sand and water having a specific gravity of about 1.7. The specific gravity of the fresh sand was 2.6. As the operation continued, portions of the fine material from the coal de-sanding screens 11, 12 and 13 were continuously withdrawn as through the hopper 17 and pipe 27. This was found to be composed of about 41% of combustible matter and possessed a specific gravity of 2.0. 5

10 This was treated by the froth flotation step. For this purpose a suspension of one part of the fine coal-sand mixture and four parts of water was treated in the froth flotation apparatus with about 2% of petroleum fuel oil under the combined effect of mechanical agitation and finely divided air bubbles. A clean sand was obtained therefrom containing only 7.5% of combustible material and having a specific gravity of 2.5, which was 15

20 returned to the fluid mass. As a by-product a fine coal was obtained from the top of the flotation apparatus containing only about 17% of ash. The fine coal particles are floated to the surface of the water in the 25

25 flotation apparatus in a froth and the froth is removed in a manner well understood by those skilled in the art. Various selective agents may be used in the flotation apparatus such as insoluble collectors and soluble 30 frothing agents. Modifying agents such as organic compounds, acids, alkalis and salts may also be used to favorably affect the surfaces of the particles in order that the finely divided coal will be more effectively preferentially floated from the sand to a point where the latter is suitable for re-use in producing the fluid mass in the separator 5. The air may be supplied to the flotation apparatus under pressure or may be beaten in 35

40 by the action of agitators. We have found that a combination of air under pressure and mechanical agitation gives very good results. The flotation step may be carried out under atmospheric pressure or under increased or diminished pressures. Instead of treating the finely divided coal and sand mixture from the screens 11, 12 and 13, substantial advantage may still be obtained by permitting the finely divided coal and sand 45

50 mixture to be returned to the separation vessel 5 and withdrawing the fine coal sand mixture from other parts of the gravity separation step in the separator 5, purifying the sand so withdrawn and then returning the same to the separator 5. It is not necessary to remove all of the finely divided coal from the sand, at least in most cases. The degree of purity of the material recovered to form the fluid mass will be governed by the special conditions controlling 55

60 the coal washing in various cases. The invention may be applied to the treatment of a great variety of coals and also for the separation therefrom of many other impurities and slate. It may be applied to the

recovery of coal or similar fuel from waste dumps of various kinds, and by the term "coal" we include such similar fuel as coke and the like.

While we prefer to use for the fluid mass 76 for the gravity separation, a mixture of sand and water, nevertheless many other finely divided materials may be used including clay, finely divided metals, ores, etc. Also while we have mentioned the use of 75 screens such as at 19 for separating slate from the sand and water and screens such as 11, 12 and 13 for separating the sized coal from the sand and water, nevertheless, any other suitable separating or classifying apparatus or devices may be used for these purposes. Before introducing the coal at 1 it may be subjected to the action of a plurality of screens, one passing all coal including pea size and smaller and the next 80 one passing only the silt. The coal above pea size may go directly to the separator 5, and likewise one half the coal held on the silt removing screen. The other half of the latter may be mixed, without cleaning, with 85 the discharge from the separator at 10. If desired soluble material may be dissolved in the water in or supplied to the separator 5 to aid in increasing the specific gravity thereof. If too much water is returned to 90 the flotation apparatus through pipe 27, a settling tank may be introduced to remove part of the water before the material is introduced into the flotation apparatus. Also if the amount of water is insufficient 95 more water may be added to pipe 27. Likewise any other suitable form of flotation apparatus may be used, and other forms of apparatus may be substituted for the screen 2 or the same omitted altogether and many 100 other changes and modifications may be made and the invention embodied in widely different forms without departing from the spirit and scope thereof in its broader aspects. Hence we desire to cover all forms 105 and modifications coming within the language or scope of any one or more of the appended claims.

What we claim as new and desire to secure by Letters Patent is:

1. The method of cleaning coal which consists in separating impurities from the coal by gravity in a liquid having a finely divided solid in suspension therein forming a liquid medium of a specific gravity between that of the coal and impurities, withdrawing 115 finely divided solid from the gravity separation and treating it by flotation to remove finely divided coal or other impurities which may have collected therein and returning 120 the cleaned solid for further gravity separation of coal from impurities.

2. The process of cleaning coal which consists in separating therefrom impurities of higher specific gravity than the coal, by 125

gravity in a fluid mass having a specific gravity between that of the coal and impurities, the fluid mass comprising an aqueous liquid carrying in suspension a finely divided solid, withdrawing finely divided solid from said gravity separation step after it has become contaminated with substantial amounts of fine coal, treating said contaminated solid by flotation to remove fine coal therefrom, and returning the cleaned solid to the gravity separation step of the process.

3. The process of cleaning coal which consists in separating therefrom impurities of higher specific gravity than the coal, by gravity in a fluid mass having a specific gravity between that of the coal and impurities, the fluid mass comprising water carrying sand in suspension, withdrawing sand from said gravity separation step after it has become contaminated with substantial amounts of fine coal, treating said contaminated sand by froth flotation to remove fine coal therefrom, and returning the cleaned sand to the gravity separation step of the process.

4. The process of cleaning coal which comprises a gravity separation of coal from impurities of higher gravity which consists in feeding said coal into an agitated mixture of a comminuted material and water composing a fluid mass of such a gravity that

the coal will float in the upper part of said fluid mass and the impurities will sink to the lower part of said fluid mass, removing the coal and impurities thus separated from said fluid mass, subjecting a part at least of said fluid mass to a froth flotation step to remove fine coal therefrom and returning the cleaned fluid mass to the gravity separation step of the coal cleaning process.

5. The process of cleaning coal containing impurities of higher specific gravity than the coal, which consists in feeding the impure coal into an agitated fluid mass comprising water and a finely divided solid in suspension therein, forming a fluid mass of such specific gravity that the coal will float in the upper part of said mass and impurities will sink to the lower part of said fluid mass, removing purified coal from the top of the mass, removing impurities from the bottom of the mass, separating purified coal from finely divided solid matter which is removed therewith, and subjecting such finely divided solid matter to flotation separation to separate therefrom finely divided coal which is retained therein from said gravity separation.

In testimony whereof we have signed our names to this specification.

CHARLES R. DOWNS.  
CHARLES H. STRANGE.